

Dec. 15, 1936.

H. M. ELSEY

2,063,992

FACSIMILE RECEPTION

Filed June 10, 1932



Fig. 1.

Fig. 2.

Fig. 4.



Fig. 3.

Fig. 5.



WITNESSES:  
*Frederick C. Williams*

INVENTOR  
*Howard M. Elsey*  
BY *Howard Elsey*  
ATTORNEY

## UNITED STATES PATENT OFFICE

2,063,992

## FACSIMILE RECEPTION

Howard M. Elsey, Oakmont, Pa., assignor to  
Westinghouse Electric & Manufacturing Com-  
pany, a corporation of Pennsylvania

Application June 10, 1932, Serial No. 616,475

4 Claims. (Cl. 204—1)

This invention relates to improvements in reception of facsimile images. Particularly it relates to obtaining permanence and clarity of image in such types of facsimile apparatus as utilize electro-chemical action for reception.

Generally, in electro-chemical types of facsimile reception, a mark is generated between electrodes that contact or "scan", a relatively moving sheet. The sheet is moistened with chemical reagents that are released by flow of current as signals are received. The release of reagents is intended to color the sheet in accordance with variations in the signal.

In the development of this art it was sufficient relatively early that the imprinted marks differ successively only in spacing. But later, to build up what are substantially photographic images, efforts were directed in addition to obtain variations in intensity, and even to record intricate tone structures. These efforts have not been entirely satisfactory. More recently, requirements for speed have complicated the problems, since the series of electro-chemical actions that occur in the receiving sheet now must correspond to signal currents that fluctuate with extreme rapidity, such as with radio transmission. Moreover, since such signal currents are of low intensity, the solution of reagents in the sheet must be sensitive to magnify even slight variations of current to appear as appreciable differences in color deposit. Hence the colorant produced must be intense in tintorial power. Besides, it must be brought to relatively insoluble condition in a short time, else it diffuses and blurs the image. Thus, clarity of image depends on numerous contributing factors.

Previously, solutions for treating facsimile sheets have included starch and potassium iodide. These form a dark blue pigment on passage of electric current, and yield sharp images; but the images lack permanence. Another solution frequently used contained essentially potassium ferrocyanide. It depended on interaction with an iron anode. The passage of electric current caused iron to dissolve from the anode; the dissolved iron then reacted with the reagent ferrocyanide to form a dark blue precipitate on the paper. However, this leaves a mark that is blurred. This blurring appears to be due largely to the fact that the iron dissolves in two forms, as ferric ion and also as ferrous ion. The ferrous ion remains in solution and diffuses away from its source so as ultimately to discolor adjacent areas and render the image indistinct.

The present invention comprises in its objects

improvement of arrangements in electro-chemical facsimile receivers, so as to produce images that are distinct, and also to obtain quick and sensitive response to slight variations of signal current. Another object is to provide facsimile solutions that yield a wide range of image tone but yet permanency of image.

According to this invention, these objects and others are accomplished by providing a scanning anode and a conducting solution that react with each other on passage of current to obtain a permanent pigment that yields sharp definition of image. Preferably this is brought about by an anode of metal having a relatively high solution potential with solvent liquid that contains reagent to convert the resulting metal ions to free metal. In further refinement of this invention, the solution may contain reagent that at once precipitates the metal ions as insoluble compounds, so as to minimize diffusion and resultant blurring of the image, and the solution may contain also reducing agent that is effective to convert this precipitated metal compound to free metal.

Reference is made to the accompanying drawing, illustrative of the principles of this invention.

In the drawing, Fig. 1 shows, in perspective, apparatus suitable for carrying out this invention;

Fig. 2 shows a representative image that is distinct over a range of tone values, but with the scanning lines somewhat exaggerated;

Fig. 3 is an enlargement of a portion of Fig. 2 showing sharpness of outline such as results in clear definition of image;

Fig. 4 shows an image illustrating the defect of indistinctness encountered in the prior art, while

Fig. 5 is an enlargement of a portion of Fig. 4, showing the blurred outline of such defective image.

Referring more particularly to the drawing, and to a preferred embodiment of this invention, for the purpose of illustration, Fig. 1 shows a facsimile receiving sheet 1, of absorbent material such as paper, drawn through a bath 2 of reagents prepared according to this invention, and then while moist drawn between electrodes 3 and 4 to form an electrolytic cell. These electrodes are connected electrically with a receiver adapted to afford a flow of direct or rectified alternating current in accordance with incoming signals. Upper electrode 3 is shown as a stationary conducting bar having a straight contact face, while

lower electrode 4 is shown as a helical conducting bar that is rotatable to afford line contact progressively along the face of upper bar 3. This progressive line contact is repeated by each revolution of the helical electrode. The helical conductor 4 rotates relatively rapidly, while the moistened sheet advances relatively slowly, so the contacts appear across the paper as a succession of closely adjacent parallel lines. Such repeated traversing of the sheet is designated as "scanning." With variations in the signal current, corresponding variations occur in the facsimile deposit along the successive lines, as is apparent from Figs. 2 or 3. The particular scanning mechanism illustrated is disclosed and claimed in a copending application, Serial No. 421,965, filed January 20, 1930 by Zworykin and Elsey. The present invention resides in the solution and electrodes, which constitute the electro-chemical portion of a facsimile receiver.

The contact face of the electrode serving as anode, shown as 3, may be considered to be of silver, to illustrate a preferred embodiment of the present invention. With flow of current through the electro-chemical cell established by the electrodes and the solution in the sheet, the anode, silver in this example, dissolves in the solution to form ions in proportion to the current. The solution is made to contain suitable conducting material to facilitate the flow of current, and also to contain reagent effective to convert the metal ions to free metal condition, and thus to form a metal precipitate that varies along the scanning line in accordance with the signal. Preferably reducing agent is utilized to form the free metal. Thus a suitable solution contains approximately:

|                             |                   |     |
|-----------------------------|-------------------|-----|
| Formaldehyde (40%) solution | cubic centimeters | 5   |
| 40 Sodium nitrate           | grams             | 50  |
| Sodium hydroxide            | do                | 4   |
| Water                       | cubic centimeters | 500 |

Such solution is suitable for facsimile reception because formaldehyde under alkaline conditions reduces silver ion almost instantly to metallic silver. The metal in precipitating is absorbed in the sheet. Thus the metal deposit forms the scanned line in distinct accordance with variations in the signal current. The speed of reduction to free metal is increased with increase in alkalinity, but if the solution is too alkaline, the paper strength deteriorates until it does not withstand the mechanical friction of the electrodes, but tears. In the solution described, the alkalinity is limited suitably to avoid tearing of such strong paper as is obtainable at this time, but it will be desirable to control the alkalinity according to the requirements in particular instances. This will vary somewhat according to the nature of the material and mechanical conditions affecting the strength of the sheet. The sodium nitrate is added to increase electrical conductivity and to impart smoothness to the electrolytic action at the cathode. Both of these sodium compounds increase electrical conductivity, and so facilitates flow of the small current involved.

A modified form of this invention is based on the observation that, although the time factor of reduction to free metal is very small with the solution described, yet during even the time that the silver ion is in solution it may diffuse away from its point of origin and so render the lines less sharp and blur the image when reduction

finally occurs. Such result is illustrated in Figs. 4 and 5. However, this invention combats lack of sharpness by adding reagents to react even more quickly, not to reduce the silver ion at once but first to form insoluble compounds with it. With the silver as insoluble compound once fixed to its point of origin, it is subsequently reduced to free metal.

Illustrative of this embodiment of the invention is a solution containing approximately:

|                           |                   |      |
|---------------------------|-------------------|------|
| Pyrocatechin              | grams             | 10   |
| Potassium bromide         | do                | 5    |
| Potassium iodide          | do                | 0.25 |
| Ammonium nitrate          | do                | 50   |
| Metol                     | do                | 1    |
| Sodium sulfite (crystals) | do                | 1    |
| Water                     | cubic centimeters | 500  |

In this case the bromide and the iodide react rapidly with the silver ion as it enters solution from the anode, to form insoluble silver bromide and iodide. It may be desirable to photosensitize these precipitates to facilitate reduction to free metal, and it may be desirable to alter the reducing agents, but from the present description, variations of this invention will be apparent to those skilled in the art. Ammonium nitrate serves to control the hydrogen ion concentration of the solution to prevent undue oxidation of the reducing agent, pyrocatechin and also markedly increases the conductivity of the solution. The nitrate ion also facilitates the reactions that occur at the cathode. The metol and the sodium sulfite also serve to protect the pyrocatechin against oxidation by the air.

Silver is preferable as anodic metal, not only because of its permanency of image, but also because silver dissolves only as univalent metal ion. This eliminates difficulties encountered with metal, such as iron, that is multi-valent, where different ions are formed at an anode in ratios that are functions of the current density. Silver also introduces a factor of considerable importance where there is but small current flow; namely, that one atomic weight of the univalent anodic metal is dissolved for each faraday of electricity flowing, while a metal of valence two or valence three would require respectively two or three faradays of electricity to dissolve an atomic weight of such metal. Moreover, iron and various multivalent metals tend to become passive; while silver, avoiding this difficulty, dissolves more consistently in proportion to the current flow.

It is within the scope of this invention to utilize as anode not only pure metal, but also alloys. One merit of alloys is greater hardness, or resistance to wear and deformation.

Also variations are contemplated in the electrolyte. For example, in lieu of pyrocatechin or of formaldehyde, gallic acid may be used, or acetaldehyde, or hydroquinine, pyrogallol, etc. The effect of these and other equivalents will now be apparent to those skilled in the art. Similarly other precipitants than potassium bromide or iodide may be used. Moreover, it is within the scope of this invention to modify the color or intensity of the metal precipitate.

Also there may be modifications in the manner of applying the reagents. For instance, the reducing agent, as pyrocatechin may be omitted from the solution with which the facsimile sheet is treated at the electrodes, but after passage of the current the sheet may be exposed to light and then treated with suitable reducing agent to

bring out the latent image. And even where pyrocatechin or the like is present during the flow of current, the image may be intensified with suitable reducing agent, or other agents known in the photographic art.

Further, the electrolyte in the paper may contain reagents to free pigmenting material at the cathode, whether or not anodic metal is reduced. For instance, with silver anode and reducing conditions as heretofore described, the solution may contain a metal salt, such that while silver is precipitating at the anode, metal is freed at the cathode. Lead, for example, forms suitable soluble salts for cathodic deposit. With the electrodes in registry, the lead remains in the paper as part of the imprinted image.

It may be desirable to modify the electrolyte so as to minimize drying of the paper, or to regulate the degree of moistness during contact with the electrodes, or to lower the freezing point of the solution to provide for reception at low temperature. Glycerine, alcohol, and sugar thus may be included in the electrolyte.

It will be understood that although this description of the invention refers to scanning lines of continuous nature, the intended purport is to include also discontinuous scanning lines, or a series of dots for example. Also the benefits of this invention extend to simple telegraph reception, as well as to more intricate facsimile reception.

It is apparent that the drawing necessarily exaggerates somewhat the intensity and spacing of the scanning lines. In actual practice, the scanning lines disappear substantially except to form the image. The usefulness of the present invention is indicated by the fact that it is capable of bringing out the image very shortly after the electrodes have moved over a given line. This facilitates immediate adjustment to correct any irregularities that may appear. The rapidity of action of this electrochemical arrangement is evident from the fact that normally about eighty scanning lines per lineal inch of receiving sheet are generated, or about one hundred twenty a minute. A normal voltage across the scanning electrode, or the "knife-edge drop", is about sixty volts with a current of about sixty milliamperes. It has been found that the deposit obtained is approximately proportional to the current, but that the pig-

mentation or intensity of image mounts in proportion to the logarithm of the current. Under these conditions adjacent areas are made distinguishably different in intensity with current flow over time intervals each of the order of 5 half a microsecond.

According to the provisions of the patent statutes, I have explained the principles and mode of operation of my invention and have described what I now consider to represent its best embodiment. However, I desire to have it understood that, within the scope of the appended claims, the invention may be practiced otherwise than as specifically described.

I claim as my invention:

1. In combination with facsimile receiving apparatus comprising scanning electrodes having a metal anode adapted to dissolve with flow of electric current and a receiving sheet of absorbent material adapted to be moved in contact with the electrodes, an alkaline electrolyte adapted to moisten the sheet and to precipitate dissolved anodic metal with flow of current through the sheet, the alkalinity of the solution being limited in accordance with the strength of the moving, moistened sheet to avoid tearing thereof.

2. In combination with a soluble metal anode for facsimile receiving to precipitate metal pigment, an electrolyte comprising alkaline material, a precipitant to form a compound with metal ions from the anode, and a reducing agent adapted to precipitate free metal from the precipitated metal compound and containing metal in solution adapted to be released as free metal.

3. In combination with a silver anode for facsimile receiving to precipitate free silver in a receiving sheet, an electrolyte comprising reagent to precipitate silver ions as dissolved from the anode, and organic reducing agent to release free silver from the precipitate, and containing metal in solution to be released as free metal in the receiving sheet.

4. In combination with a silver anode for facsimile receiving to precipitate free silver in a receiving sheet, an electrolyte comprising, organic reducing agent, soluble halide, ammonium nitrate and alkali metal sulphite.

HOWARD M. ELSEY.

50